

## UNITED STATES PATENT OFFICE.

ALAN KISSOCK, OF LOS ANGELES, CALIFORNIA.

## PROCESS OF RECOVERING TIN.

No Drawing.

Application filed June 15, 1921. Serial No. 477,788.

*To all whom it may concern:*

Be it known that I, ALAN KISSOCK, a citizen of the United States, residing at Los Angeles, in the county of Los Angeles and 5 State of California, have made certain new and useful Improvements in Processes of Recovering Tin, of which the following is a specification.

The invention relates to a novel detinning process, that is, a process for recovering the tin coating from what is usually known as "tin scrap."

The invention consists in the novel steps, sequence of steps, sub-processes and processes herein described. The objects and advantages of the invention will be set forth in part hereinafter, and in part will be apparent to those skilled in the art, or may be learned by practicing the invention.

10 In commercial work the tin scrap usually comes in bales, and a concrete or iron vat or somewhat shallow tank is usually employed for the first or chemical part or step in the process.

15 In carrying out my process, the tin scrap is immersed in an alkaline polysulfide solution, and at the present time I preferably employ sodium polysulfide, largely for economic reasons. This solution in my present 20 practice consists preferably and approximately of 4 pounds of sodium polysulfide dissolved in about 2 gallons of water, although these proportions under different conditions of practice may be varied very 25 widely.

By the action of this solution on the tin scrap, the tin coating is completely dissolved from its sheet iron or sheet steel base, with the formation of a soluble alkali thio-

30 stannate.

The reaction is probably as follows:—



or



35 Although iron and steel are ordinarily unattacked by such alkaline sulfide solutions, usually in practice a certain small proportion of the iron or steel of the tin scrap, 40 which is in contact with the tin, is attacked to some degree by the solution, with the formation of an insoluble iron sulfide, which readily oxidizes to a basic iron sulfate.

To recover the metallic tin from the alkali 45 thio-stannate solution, when the solution as made up has become, through the operation

of the process, impregnated with the tin to its full or to a sufficient extent, the basic iron sulfate is separated from the solution by filtration, and the clear solution of alkaline (in the present instance, sodium) thio-stannate is electrolyzed by means of a low voltage current.

The anode or anodes employed are preferably of insoluble or substantially insoluble 50 material, such as iron or graphite, and the cathode or cathodes are preferably of sheet tin, the tin from the solution being deposited on the tin cathodes. These cathodes are later melted and cast into pure block tin ingots. 55

The principal reaction is probably substantially as follows:—



The secondary reactions occurring during the electrolysis cause the appearance of sulfur at the anode, which is again dissolved by, or recombined with, the alkali hydrate 85 formed at the cathode. In this way, during the process of recovering the tin, the alkaline polysulfide is regenerated, and the thus regenerated solution is ready for the treatment of fresh tin scrap. 90

The regenerative reaction of the solution just described, is probably substantially as follows:—

Same as immediately above or eliminating 95 secondary reactions,



The process may employ the polysulfide solution either hot or cold, and the solution may be concentrated or diluted, these factors 100 or conditions only or mainly affecting the rapidity of the reaction, and it will be understood that the proportions given hereinbefore are merely illustrative of what is now regarded as good commercial practice. 105

Notwithstanding the regenerative feature of the process, addition of fresh chemicals must be made from time to time to compensate for the mechanical losses of the solution due to dipping the scrap and other features 110 of handling. The tin scrap after being subjected to the polysulfide bath whereby the

tin coating is removed therefrom, is washed to remove from such de-tinned scrap the tin-bearing solution.

The process is simple, rapid, relatively inexpensive and regenerative, besides possessing other advantages. It will be understood that changes may be made in the manner of practicing the invention within the scope of the appended claims without departing from the principles of the invention and without sacrificing its chief advantages.

What I claim is:—

1. The process of recovering tin from tin scrap which comprises acting on the tin scrap by an alkaline polysulfide solution to create an alkali thio-stannate solution and electrolyzing the alkali thio-stannate solution to deposit the tin from the solution, and thereby regenerating the solution to produce a polysulfide for use in the first step of the process.

2. The process of recovering tin from tin scrap which comprises acting on the tin scrap by an alkaline polysulfide solution to create an alkali thio-stannate solution and 25 electrolyzing the alkali thio-stannate solution by using a substantially insoluble anode to deposit the tin from the solution, and thereby freeing the tin and regenerating the polysulfide for use in the first step of the 30 process.

3. The process of recovering tin from tin scrap which comprises treating the tin scrap with an alkaline polysulfide solution to reduce the tin of the scrap to a dissolved 35 thio-stannate, electrolytically depositing the tin from the thio-stannate solution and thereby regenerating the polysulfide solution for use in the first step in the process.

In testimony whereof, I have signed my 40 name to this specification.

ALAN KISSOCK.